

## UNITED STATES PATENT OFFICE

2,553,937

## METHOD OF ELECTROLYTICALLY POLISHING ALUMINUM AND ITS ALLOYS

*Gravure*  
*Phosphoric*

Jos Patrie, Chambéry, France, assignor to Compagnie de Produits Chimiques et Electrométallurgiques Alais, Froges et Camargue, Paris, France, a corporation of France

No Drawing. Application January 11, 1949, Serial No. 70,364. In France January 17, 1948

4 Claims. (Cl. 204—140.5)

1

It is known to produce surfaces having a high reflective capacity on aluminum and aluminum alloys by the use of electrolytic burnishing or polishing methods. In such methods the part to be burnished is used as an anode in a successive series of electrolytic baths; one of those baths is called a burnishing bath and produces the burnishing effect proper, with or without a polishing action; a subsequent bath may be called a "re-enforcing" bath and serves to protect the burnished metal with a transparent film of oxide.

The steps in the treatment may for example include:

- (1) Thorough mechanical buffing;
- (2) Cleaning with a solvent or by electrolysis;
- (3) Electrolytic burnishing, during which a first film of oxide is formed;
- (4) Dissolving said initial oxide film in a phospho-chromic mixture;
- (5) Washing in tap-water.
- (6) Reenforcement in any one of the usual oxidising baths.
- (7) Rinsing in tap-water.
- (8) Dyeing.
- (9) Filling-in the pit-holes.
- (10) Brightening.

My present invention is more especially concerned with the electrolytic burnishing step. While a number of suitable baths are already known some of which are employed on a commercial scale, in practice they all show serious shortcomings. Thus some of the known baths are only satisfactory when operated in connection with high-purity aluminum, whereas others on the other hand are successful only when used on aluminum alloys; in most cases moreover the operating temperature of known baths is high, being close to 100° C. Another drawback of a number of known baths is that the current density usable therein is too low to permit a rapid burnishing process. Then again, they may require a thorough mechanical buffing treatment prior to the electrolysis treatment. Another frequent drawback is that only one face of the part to be burnished may be treated at a time or defects may arise as a result of the treatment, due for instance to a regular discharge of gases. Finally, known baths may comprise rare and expensive constituent materials, or substances dangerous to handle.

I have now discovered that through the use of certain classes of electrolytic baths, part or all of the above shortcomings of prior baths may be eliminated and a more convenient and simplified electrolytic burnishing treatment provided for

2

industrial use on aluminum and aluminum containing alloys.

According to the invention, there is provided an electrolyte for electrolytic burnishing of aluminum and its alloys, which comprises as main constituents nitric acid and water. The bath may contain only nitric acid and water. Or alternatively I have obtained satisfactory results by adding to the nitric bath an acid or a mixture of acids having a high alumina-dissolving capacity. Thus excellent results have been obtained when adding phosphoric acid to the nitric bath. Still more satisfactory results may be attained by adding to the nitric bath a mixture of phosphoric and chromic acids.

I have obtained a handsome polish and burnishing effect when maintaining the operative conditions within the following ranges:

(1) the nitric acid content within an approximate range from 5% to 65% when a nitric bath is used without any added acid or mixed acids;

(2) when only phosphoric acid is added to the nitric bath, the following approximate ranges of compositions are preferably maintained:

20 Nitric acid \_\_\_\_\_ from 30% to 45%  
Phosphoric acid \_\_\_\_\_ from 13% to 34%  
Water \_\_\_\_\_ as required to make 100%

(3) When a mixture of phosphoric acid and chromic acid is added to the nitric bath, the approximate preferred ranges are as follows:

30 Nitric acid \_\_\_\_\_ from 35% to 45%  
Phosphoric acid \_\_\_\_\_ from 8% to 24%  
Chromic acid \_\_\_\_\_ from 3% to 10%  
35 Water \_\_\_\_\_ as required to make 100%

In the above tabulations and those to follow the percentages are by weight and the acids used are assumed to be anhydrous. In practice we may use:

40 Nitric acid at 36° Baumé, specific gravity  $d=1.332$ , containing 52% by weight of nitric acid.

Nitric acid at 40° Bé., specific gravity  $d=1.333$ , containing 62% by weight of nitric acid; this type of acid is used where the bath contains over 52% nitric acid.

Nitric acid at 42° Bé., specific gravity  $d=1.41$ , containing 92.76% by weight nitric acid; this is used where the bath contains over 62% nitric acid.

50 Phosphoric acid at 59° Bé., specific gravity  $d=1.691$ , containing 87% by weight phosphoric acid.

According to aspects of the invention, the following preferred operative conditions are em-

ployed when using the improved electrolysis bath:

(1) the bath is operated at surrounding temperature. Preferably the temperature is maintained under 20° C.

(2) A high degree of agitation is necessary to obtain good results. Thus insufficient agitation or non-uniform agitation will produce on the aluminum surfaces reflection-distorting fleece-like effects.

(3) The current density may be varied in the range of from about 90 to about 450 amperes per square foot with a corresponding time range of from about 10 to about one or two minutes, according to the current density and the initial surface condition of the articles.

The cathode used in the improved bath is an aluminum or a graphite cathode. The tanks or containers containing the bath may be made of stainless steel, various plastics, ebonite-coated iron or generally any suitable materials impervious to the acids used in my process. Cooling means should be provided, since heat is rapidly evolved in the bath and, as stated, the temperature thereof should not exceed about 20° C. in operation.

The steps prior to and the steps subsequent to the burnishing step may be accomplished in any of the well-known ways. Thus for the solvent-cleaning operation, a substance such as trichloroethylene or the like may be used. If the cleaning operation is to be carried out by electrolysis, I may use, for example, a bath of the following composition:

|                               | Grams |
|-------------------------------|-------|
| Anhydrous trisodium phosphate | 100   |
| Anhydrous sodium carbonate    | 200   |
| Soda silicate                 | 5     |

This bath is used at about 20° C. temperature with direct current. The articles to be cleaned are placed as a cathode.

The voltage is about 12 volts and the current density from about 45 to 110 amperes/sq. ft., depending on the type of alloy from which the articles are made. The duration of the treatment may be of about 2 or 3 minutes.

The initial oxide film to be formed during the burnishing step may be dissolved, for instance by means of a phospho-chromic bath containing:

Phosphoric acid: 360 cc. of an 87% H<sub>3</sub>PO<sub>4</sub> solution (d=1.691)  
Chromic acid: 180 grams  
Water: 640 cc.

The reenforcing treatment may comprise an anodic oxidisation in an aqueous bath containing 20% of its weight of 36° Bé. sulphuric acid. This bath may be used at a temperature of about 20° C. with a current density of about 13.8 amperes/sq. ft.

Some examples will now be given of typical bath compositions according to the invention together with the conditions used in operating them:

**Example 1.—Nitric acid, 6.5%**

Water: 93.5%

Conditions of operation:

Temperature: 20° C.

Voltage: 3 volts

Curr. density: 186 amp./sq. ft.

The time of treatment is from about 10 to 15 minutes, during which strong agitation is maintained.

The bath of this example is particularly suitable for high purity aluminum.

**Example 2.—Nitric acid: 62%**

Water: 38%

Conditions of operation:

Temperature: 20° C.

Voltage: 4 v.

Current density: 280 amp./sq. ft.

The time of treatment is from about 10 to 15 minutes, with strong agitation throughout.

The bath of this example is especially suitable for high-purity aluminum.

**Example 3.—Nitric acid: 41.5%**

Phosphoric acid: 17.5%

Water: 41.0%

Conditions of operation:

Temperature: 10 to 20° C.

Voltage: 3 to 7 v.

Current density: 186 to 370 amp./sq. ft.

Strong agitation is maintained throughout the process.

The bath of this example is capable within a few minutes to burnish aluminum of high purity as well as ordinary grades of aluminum and aluminum alloys.

**Example 4.—Nitric acid: 41%**

Phosphoric acid: 14

Chromic acid: 5

Water: 40

Conditions of operation:

Temperature: 10 to 20° C.

Voltage: 3 to 7 v.

Current density: 186 to 370 amp./sq. ft.

The bath of this example burnishes in a few minutes aluminum of high purity as well as ordinary grades of aluminum and aluminum alloys.

The above examples are given merely by way of indication and not of limitation, and it is to be understood that many modifications may be made therein without exceeding the scope of the invention.

The use of my improved bath results in the following advantages:

(1) The articles to be burnished do not require to be subjected prior to burnishing to a thorough mechanical buffing, since the bath is effective to produce in addition to burnishing, a slight polishing or buffing effect. It is merely necessary to effect a rough mechanical polish in order to remove the coarser asperities from the surface, such as scratches and surface irregularities found in metal castings direct from the foundry.

(2) The improved bath burnishes at room temperature. The fact that it is operative under 20° C. forms one of the most remarkable characteristics of the present invention. Thus it will not be required to provide, as in the conventionally used methods, heating means for the bath container, and this will substantially reduce cost of the plant installation. Moreover the cost of operation of the process is also substantially lowered since it is no longer necessary to hold the bath at high temperature.

(3) The articles treated are polished and burnished on both faces and their appearance is not marred by the presence of stripes due to regular discharge of gases. This advantage is particularly appreciable in connection with the manufacture of articles used for ornamental purposes.

(4) Use of my improved bath makes it possible to operate under a very low voltage (about 3 to 7 volts) whereby the item relating to electric

energy consumption in the over-all cost price will be notably diminished.

(5) The substances used in the composition of the bath are widely available, and may be handled without any exceptional precautions.

(6) The bath is applicable for burnishing both aluminum of high purity and of ordinary grades, as well as aluminum base alloys.

Among the aluminum base alloys in connection with which my improved electrolytic burnishing bath is applicable, I may mention aluminum alloys containing copper (such as duralumin), magnesium (such as aluminum alloys containing from 3 to 5% magnesium), magnesium and silicon containing alloys such as almasilium, and aluminum alloys containing magnesium and zinc. A handsome burnish may also be obtained on aluminum alloys of the moldable type, such as those containing from 3 to 5% magnesium, the alloy known as "A. P. M." (4.2% Cu, 0.18-0.40% Mg, 0.17-0.35% Ti), the alloy known as "Y" (3.6-4.5% Cu, 1.2-1.8% Mg, 1.7-2.3% Ni) and others.

What I claim is:

1. In a method for electrolytically polishing and brightening articles consisting at least for the major part of aluminum, the step of effecting the electrolytic polishing and brightening treatment at a temperature below 20° C. in an electrolysis bath containing 30 to 45% by weight of nitric acid and a significant amount of at least one member of the group consisting of phosphoric and chromic acids, the total of the acids ranging between 43 and 79% by weight, the balance being water.

2. In a method for electrolytically polishing and brightening articles consisting at least for the major part of aluminum, the step of effecting the electrolytic polishing and brightening treatment under a current tension of 3 to 7 volts and

at a current density of 10 to 50 amperes per square decimeter, and at a temperature below 20° C. in an electrolysis bath containing 30 to 45% by weight of nitric acid and a significant amount of at least one member of the group consisting of phosphoric and chromic acids, the total of the acids ranging between 43 and 79% by weight, the balance being water.

3. In a method for electrolytically polishing and brightening articles consisting at least for the major part of aluminum, the step of effecting the electrolytic polishing and brightening treatment at a temperature below 20° C. in an electrolysis bath containing 30 to 45% by weight of nitric acid and 13 to 34% by weight of phosphoric acid, the balance being water.

4. In a method for electrolytically polishing and brightening articles consisting at least for the major part of aluminum, the step of effecting the polishing and brightening treatment at a temperature below 20° C. in an electrolysis bath containing 35 to 45% by weight of nitric acid, 8 to 24% by weight of phosphoric acid, and 3 to 10% by weight of chromic acid, the balance being water.

JOS PATRIE.

#### REFERENCES CITED

30 The following references are of record in the file of this patent:

#### UNITED STATES PATENTS

| Number    | Name      | Date          |
|-----------|-----------|---------------|
| 2,462,197 | Jernstedt | Feb. 22, 1949 |

#### FOREIGN PATENTS

| Number  | Country       | Date          |
|---------|---------------|---------------|
| 504,026 | Great Britain | Apr. 17, 1939 |
| 798,721 | France        | Mar. 11, 1936 |